

106. COMPOSITIONS,  
COATING OR PLASTIC.

844,668

98 Date, 102, 646, July 29, 1884 (106-45)

|               |     |
|---------------|-----|
| Sand          | 85% |
| Hydrated Lime | 10% |
| Cement        | 5%  |

## UNITED STATES PATENT OFFICE.

LAURENCE ELKUS, OF INDIANAPOLIS, INDIANA.

## COMPOSITION FOR BRICKS.

No. 844,668.

Specification of Letters Patent.

Patented Feb. 19, 1907.

Application filed June 1, 1906. Serial No. 319,756.

*To all whom it may concern:*

Be it known that I, LAURENCE ELKUS, of the city of Indianapolis, county of Marion, and State of Indiana, have invented a new and useful Improvement in Bricks, of which the following is a full, clear, and exact description.

The object of my invention is to provide a brick having ability to resist dampness, moisture, and fire to a greater degree than those heretofore known.

The composition consists in mixing sand, cement, and lime in approximately the following proportions: sand, eighty-five per cent., (85%); hydrated lime, ten per cent., (10%); cement, five per cent., (5%). I do not wish, however, to be confined to these exact proportions, as they may vary to the extent of three per cent., (3%), greater or less, of cement and three per cent., (3%), greater or less of lime.

The process of manufacture is as follows: The sand is introduced into a steel cylinder, where it is thoroughly dried. Lime is pulverized and slaked in a cylinder or other machine. The hydrated lime, with the dried

sand, is then mingled in a tube-mill with ground cement and thence discharged into a wet mixer, consisting of a revolving pan with drop-bottom and paddles so arranged as 30 thoroughly to agitate the mixture. Arrangement is made to spray water on this mixture. From the mixer the moist material is taken to the press, where it is pressed into molds the size of bricks. The soft 35 bricks are then taken to the hardening-cylinders and are hardened under a steam-pressure. While in the hardening-cylinders steam-pressure of about one hundred and fifty pounds to the square inch is introduced, 40 and this steaming continues for eight hours.

What I claim as my invention, and desire to secure by Letters Patent, is—

In an artificial stone the combination of sand, hydrated lime and cement in substantially the proportions specified. 45

In witness whereof I have hereunto set my hand this 28th day of May, 1906.

LAURENCE ELKUS.

In presence of—

ETHEL KENNARD,  
CHAS. S. SYMONS.